

[54] TANTALUM BASE ALLOYS

[75] Inventor: Raymond W. Buckman, Jr.,  
Pittsburgh, Pa.[73] Assignee: Westinghouse Electric Corporation,  
Pittsburgh, Pa.

[22] Filed: Oct. 30, 1968

[21] Appl. No.: 771,714

**Related U.S. Application Data**[63] Continuation-in-part of Ser. No. 598,941, Dec. 5,  
1966, abandoned, which is a continuation-in-part of  
Ser. No. 454,650, May 10, 1965, abandoned.

[52] U.S. Cl. .... 75/174, 148/32

[51] Int. Cl. .... C22c 27/00, C22f 1/18

[58] Field of Search .... 75/174; 148/32, 32.5, 133

[56] **References Cited****UNITED STATES PATENTS**3,379,520 4/1968 Chang et al. .... 75/174  
3,390,983 7/1968 Ammon et al. .... 75/174**OTHER PUBLICATIONS**

Ammon et al., "Pilot Production and Evaluation of

Tantalum Alloy Sheet," WAN-LPR-M-004, June 15,  
1963, relied on pages 50, 51, 53, 55, 58, 62, 78, 79 &  
80.ASD-TDR-62-594, "Investigation of Tantalum and  
Its Alloys," May 1963, relied on pages 93, 95, 96,  
101, 103, 104, 107 & 108.*Primary Examiner*—Charles N. Lovell  
*Attorney, Agent, or Firm*—F. Shapoe; R. T. Randig[57] **ABSTRACT**

This invention is directed to tantalum-base alloys having superior elevated temperature strength and high resistance to creep deformation at elevated temperature in a high vacuum or space environment. The alloys comprise from 4 to 8.5 percent tungsten, up to 3 percent of at least one of the group consisting of molybdenum and rhenium, up to 1.5 percent of at least one of the group consisting of zirconium and hafnium, up to 0.04 percent of at least one of the group consisting of carbon and nitrogen and the balance essentially tantalum.

**9 Claims, 3 Drawing Figures**

PATENTED FEB 12 1974

3,791,821



FIG. 2.



FIG. 3.

WITNESSES

Theodore T. Krikel  
James T. Young

INVENTOR

Raymond W. Buckman, Jr.  
BY  
Robert W. Bandy  
ATTORNEY

## TANTALUM BASE ALLOYS

This application is a continuation-in-part of application Ser. No. 598,941, filed Dec. 5, 1966, now abandoned, which in turn was a continuation-in-part of application Ser. No. 454,650, filed May 10, 1965, now abandoned, assigned to the same assignee as the present invention.

The invention described herein was made in the performance of work under a NASA contract and is subject to the provisions of Section 305 of the National Aeronautics and Space Act of 1958, Public Law 85-568 (72 Stat. 435; 42 U.S.C. 2457).

The development of reliable space power generation systems requires the availability of alloys which can withstand the rigorous environment in which they are to be used, namely high operating temperatures, near-vacuum pressures, high operating stresses and the corrosive effect of liquid alkali metals. The alloys employed for the tubing and sheet for such space power systems are required to have a combination of characteristics including good fabricability, good weldability, strength at elevated temperatures, good resistance to creep deformation at elevated temperatures in high vacuum and corrosion resistance to liquid alkali metals.

Tantalum-base alloys containing reactive metal additions such as zirconium and hafnium have been and are presently under development in the industry and such alloys exhibit good fabricability and corrosion resistance to liquid alkali metals. These alloys were designed primarily for short-time applications; that is, for periods of use amounting to about ten hours, where solid solution alloy additions are extremely beneficial in that they confer high tensile strength upon the alloys. High tensile strength, however, is not necessarily indicative of good resistance to creep deformation. This is particularly true where the operating environment in which the alloy is expected to function is a high vacuum, for it is known that the environment pressure has a significant effect on creep properties, and, in some cases, high vacuum reduces resistance to creep deformation.

Accordingly, it is an object of this invention to produce fabricable tantalum-base alloys which are resistant to the corrosive effect of liquid alkali metals and have good strength at elevated temperatures and high resistance to creep deformation at elevated temperature in a vacuum environment.

A more specific object of the present invention is to provide a tantalum-base alloy having dispensed secondary phases comprising a major proportion of dimetal carbides and reactive metal nitrides and which is characterized by improved creep resistance, good fabricability and weldability and a controlled ductile-brittle transus temperature below room temperature.

Other objects of this invention will become apparent to those skilled in the art when taken in conjunction with the following description and the drawings, in which:

FIG. 1 is a portion of the pseudo-ternary phase diagram of the tantalum rich corner of the (Ta + W + Re)-Hf-C alloys at the 1315°C (2900°F) isotherm;

FIG. 2 is a graph illustrating the time to 1 percent total strain versus the hafnium plus zirconium content

and carbide character under a stress of 15K psi and in a vacuum of  $1 \times 10^{-8}$  Torr; and

FIG. 3 is a graph illustrating the time to 1 percent total strain versus the rhenium content in tantalum base alloys tested under the same conditions as the alloys of FIG. 2.

The tantalum-base alloys of this invention contain a dispersed secondary phase comprising complex carbides or nitrides or both which serve to pin dislocations and thus greatly improve the resistance of alloy member to creep deformation. Characteristically, the carbide phases which are formed in the alloy of the present invention, as circumscribed by the appended claims, have a close packed hexagonal crystallographic configuration with lattice constants substantially within the range between about,  $a_0$ , 3.10 to about 3.14 Å. and,  $c_0$ , about 4.92 to about 4.96 Å. These lattice parameters confirm that there is only minor substitution of hafnium and/or tungsten for tantalum in the formation of the dimetal carbide having the general formula  $(Ta, Hf, Mo, Re, Zr, W)_2 C_{1-x}$  where  $x$  is substantially less than 1 and approaches zero. When the composition is maintained within the limits set forth hereinafter the preferred dimetal carbide is formed as will be evident from inspection of FIG. 1.

The alloys of the invention include, in addition to tantalum, the element tungsten and some or all of the elements molybdenum, rhenium, hafnium, zirconium, carbon, and nitrogen.

Broadly stated, these alloys comprise, by weight, from 4 percent to 8.5 percent tungsten, at least one element selected from the group consisting of molybdenum and rhenium, molybdenum when present amounting to up to 1.25 percent, rhenium when present amounting to up to 3 percent, the total amount of molybdenum plus rhenium being at least 0.5 percent, but not exceeding 3 percent, up to 0.75 percent zirconium, up to 1.5 percent hafnium, the total of zirconium and hafnium not exceeding 1.5 percent, trace amounts to about 0.03 percent nitrogen, trace amounts to about 0.03 percent carbon, the total carbon and nitrogen being at least about 0.01 percent but not exceeding about 0.04 percent, and the balance essentially tantalum, except for incidental impurities.

Each of the alloying components performs a specific function within the alloy of the present invention. Thus tungsten within the stated range improves the strength of the solid solution. It is desired to maintain at least 4 percent for effective solid solution strengthening. Where the tungsten content is increased to beyond about 8.5 percent the fabricability properties and especially weldability appear to deteriorate. Up to about 1.25 percent molybdenum and up to about 3.0 percent rhenium may also be present to aid in the solid solution strengthening; however, such additions must be carefully balanced in order to obtain an outstanding combination of properties. This is clearly demonstrated by reference to FIG. 3.

It is noted in FIG. 3 that where the rhenium content is increased up to about 0.5 percent the creep properties are vastly improved. Further increases in the rhenium content provide only a smaller improvement in the creep properties up to about 3.0 percent rhenium. However while the creep properties are improved the as-welded ductility as exemplified by the ductile-brittle transition temperature (DBTT) is raised from about -225°F at the 1 percent rhenium level to about room

temperature for rhenium contents of about 3 percent. Consequently, the preferred rhenium content lies within the range between about 0.5 percent and about 1.5 percent although useful alloys can be produced over the entire range depending upon the ultimate requirements in use.

The alloy of the present invention also contemplates the presence of reactive metals hafnium and zirconium with the hafnium being the preferred component for obtaining optimum fabricability and weldability. No substantial difference appears to exist between hafnium and zirconium insofar as the creep properties are concerned. Up to 0.75 percent zirconium may be present and up to 1.5 percent hafnium can be present with the proviso that the sum of the zirconium plus hafnium does not exceed 1.5 percent. The reason for these limits appear hereinafter.

Hafnium and zirconium, while entering into solid solution can also react with the carbon present to form a series of carbides depending upon the amount of reactive metal and carbon which is present. The higher amounts of hafnium and/or zirconium necessary to stabilize the monometal carbide is effective for exerting a powerful influence upon the creep properties of the alloy of this invention.

Referring now to FIG. 2, the effect of the hafnium and zirconium on the creep properties is illustrated. Thus where the hafnium and zirconium are maintained within the limits set forth it may be observed the alloy will possess good creep properties. Where however, the upper limit is exceeded a marked deterioration in the creep properties is evident. The limits of the phase boundaries set forth in FIG. 1 as respects the crystallographic character of the carbides present are also shown in FIG. 2. Thus it will become apparent that in order to obtain outstanding creep properties only the dimetal carbide should be present. Accordingly, the limits set forth hereinbefore for the hafnium and zirconium have been selected so that only the dimetal carbide is present in the alloy of the present invention.

In addition to limiting the solution strengthening components to the limits set forth hereinbefore, it is also preferred to limit the total solute components to a maximum of 10 percent, that is, the sum of the tungsten, molybdenum, rhenium, hafnium and zirconium must be limited to 10 percent with the individual components also being limited to each of their respective ranges.

The alloy of the present invention envisages the presence of nitrogen in amounts of up to 0.03 percent and carbon in amounts of up to 0.03 percent with the total carbon and nitrogen limited to 0.04 percent maximum. Both carbon and nitrogen react to form carbides, nitrides and carbonitrides. Of primary importance, however, the phases so formed must exhibit a major proportion of the dimetal carbide in order to obtain optimum creep properties. By inspection of FIG. 1 it will be observed that only the dimetal carbide phase is present when the alloy composition is balanced as described hereinbefore.

Reference is again directed to FIG. 3 which also demonstrates the effect of carbon and nitrogen on the creep properties. Thus in FIG. 3 the curve 10 illustrates the level of properties where the carbon plus nitrogen content is less than 50 ppm whereas curve 12 illustrated

the level of properties where the carbon plus nitrogen is within the range between 200 and 300 ppm. FIG. 3 clearly demonstrates that where the dispersed secondary dimetal carbide phase is present, outstanding creep results are obtained by controlling the alloying components as set forth hereinbefore.

One particularly useful group of alloys of this invention contains the above specified elements in the ranges of, by weight, from 4 percent to 8 percent tungsten, 10 from 0.5 percent to 1.25 percent molybdenum, from 0.5 percent to 2.5 percent rhenium, from 0.1 percent to 1.5 percent hafnium, from trace amounts to 0.75 percent zirconium, the total of zirconium and hafnium not exceeding 1.5 percent, trace amounts to 0.03 percent carbon, from 0.01 percent to 0.03 percent nitrogen, the total carbon and nitrogen being at least 0.01 percent but not exceeding 0.04 percent, and the balance essentially tantalum with small amounts of incidental impurities. Another preferred composition 15 within these ranges comprises, in weight percent, about 5.5 percent to 5.8 percent tungsten, from about 0.6 percent to 0.9 percent molybdenum, about 1.4 percent to 1.6 percent rhenium, about 0.2 percent to 0.3 percent hafnium, about 0.1 percent to 0.2 percent zirconium, about 0.02 percent carbon, about 0.02 percent 20 nitrogen and the balance essentially tantalum with small amounts of incidental impurities. Expressing the composition of this preferred alloy in atomic percent the tungsten amounts to about 5.6 at %, the molybdenum about 1.4 at %, the rhenium about 1.5 at %, the hafnium, zirconium, carbon and nitrogen are present in equal amounts, that is about 0.25 at %.

Still another preferred composition comprises, in weight percent, from about 7 to 8.5 percent tungsten, 35 from 0.5 to 1.5 percent rhenium, from 0.5 to 1.25 percent hafnium, from 0.02 to 0.03 percent carbon and the balance essentially tantalum with small amounts of incidental improvements.

A specific outstanding alloy composition comprises, 40 by weight, about 8 percent tungsten, about 1 percent rhenium, about 0.7 percent hafnium, about 0.025 carbon and the balance essentially tantalum. In this alloy nitrogen is substantially absent. The creep rate properties, namely time to 1 percent strain at elevated temperatures under high loads in a high vacuum, have proven to be outstanding. Because of fabricability properties superior to any of the other alloys of this invention, this composition is particularly advantageous.

50 Other desirable alloy compositions within the scope of the invention comprise, by weight, about 6.3 percent to 7.2 percent tungsten, one element selected from the group consisting to about 0.7 percent to 1 percent, rhenium, when present amounting to about 1.4 percent to 1.6 percent, about 0.2 percent to 0.3 percent zirconium, up to about 0.4 percent to 0.6 percent hafnium, about 0.02 percent nitrogen, up to about 0.02 percent carbon and the balance tantalum except for incidental impurities.

60 Alloys of the invention were prepared having the compositions set forth in Table I. Table I also includes the composition of the highly meritorious tantalum-base alloy known in the art as T-222 alloy for comparative purposes. The quantities of each element are expressed in weight percent in the Table.

TABLE I

| Alloy | W   | Mo   | Re   | Zr   | Hf  | C    | N   | Ta   |
|-------|-----|------|------|------|-----|------|-----|------|
| A     | 5.7 | 0.7  | 1.56 | 0.13 | .25 | .017 | .02 | Bal. |
| B     | 7.1 | —    | 1.56 | 0.26 | —   | *    | .02 | Bal. |
| C     | 7   | 0.85 | —    | 0.26 | —   | *    | .02 | Bal. |
| D     | 6.5 | 0.8  | —    | 0.26 | 0.5 | .017 | .02 | Bal. |
| E     | 8   | —    | 1    | —    | 0.7 | .025 | —   | Bal. |
| F     | 9   | —    | —    | —    | 1   | .025 | —   | Bal. |
| T-222 | 10  | —    | —    | —    | 2.5 | .01  | —   | Bal. |

\* residual carbon level 2-30 ppm.

Each of the exemplary alloys A, B, C, D and E of Table I has substantial merit in its own right. Each of these alloys is representative of a different type of alloy within the broad invention. Compositions of the Alloy A and Alloy E type have been more generally defined above as preferred compositions. Set forth below are definitions of each of the more limited ranges, within the broad range, of the alloy types represented by Alloys B, C and D.

Thus, desirable alloys of the Alloy B type have the compositions of, by weight, about 6.8 percent to 7.2 percent tungsten, about 1.4 to 1.6 percent rhenium, about 0.2 to 0.3 percent zirconium, about 0.02 percent nitrogen, and the balance tantalum.

Compositions of the Alloy C type have substituted therein about 0.7 to 1.0 percent molybdenum for all of the rhenium in the Alloy B type, but are otherwise of similar composition.

Compositions of the Alloy D type contain about 6.3 to 7.2 percent tungsten, about 0.7 to 1.0 percent molybdenum, about 0.2 to 0.3 percent zirconium, about 0.4 to 0.6 percent hafnium, about 0.02 percent carbon, about 0.02 percent nitrogen, the total carbon and nitrogen not exceeding 0.04 percent, and the balance tantalum.

Reference is directed to Table II which lists the tensile test results for the compositions set forth in Table I. Included in Table II are test results for two compositions Alloy F and Alloy T-222 each of which is outside the scope of the present invention.

From the above short time data it is seen that alloys A, B, C and D of this invention are equal or somewhat superior to the alloy T-222 in strength at the 2400°F temperature level while retaining ductility to an acceptable degree. Alloy E is somewhat lower in strength than the T-222 alloy, but equal to or better than T-222 alloy in ductility.

The materials tested above were obtained from non-consumable arc melted material. However, material of similar quality can also be produced by consumable arc melting or electron beam melting techniques as well. In any case, the raw materials used are of high purity; for example, the tantalum employed 99.9 percent pure with no more than 20 ppm each of the relatively volatile impurities Fe, Si, Cr and Pb. The tungsten and molybdenum used were also over 99.9 percent pure. The hafnium used contained as much as 2.5 percent by weight of zirconium. The as-melted alloys contain 20 to 100 ppm each of carbon and nitrogen without intentional addition thereof. The as-melted material in the case of Alloys A, B, C and D, was annealed one hour at 2300°C then upset forged to a 50 percent reduction at 1200°C. In the case of Alloy E, the as-melted ingot was forged to 70 percent reduction at 1400°C. Excellent forgeability characteristics were exhibited under the described conditions. Generally the forging is carried out in the temperature range from 1200° to 1400°C. The upset forged slab was annealed one hour at 1650°C and then was cold rolled 80 percent with excellent quality strip being obtained. The weldability of

TABLE II

| Alloy | Test Temperature (°F) | Tensile Properties<br>(Tested In The As-Worked Condition) |                                 |      | Percent Elongation |
|-------|-----------------------|-----------------------------------------------------------|---------------------------------|------|--------------------|
|       |                       | 0.2% Offset Yield Strength (psi)                          | Ultimate Tensile Strength (psi) |      |                    |
| A     | R.T.                  | 160,200                                                   | 168,700                         | 3    |                    |
|       | R.T.(1)               | 127,100                                                   | 134,000                         | 24   |                    |
| B     | 2000                  | 95,300                                                    | 98,800                          | 3.90 |                    |
|       | 2400                  | 66,200                                                    | 72,700                          | 6.60 |                    |
| C     | R.T.(1)               | 106,600                                                   | 118,500                         | 26   |                    |
|       | 2400                  | 61,300                                                    | 67,900                          | 6    |                    |
| D     | R.T.(1)               | 101,000                                                   | 111,700                         | 26   |                    |
|       | 2400                  | 77,600                                                    | 80,100                          | 5    |                    |
| E     | R.T.(1)               | 59,200                                                    | 61,100                          | 7    |                    |
|       | 2400(1)               | 85,000                                                    | 105,400                         | 25.9 |                    |
| F     | R.T.(1)               | 35,400                                                    | 40,900                          | 35   |                    |
|       | 2400(1)               | 78,600                                                    | 106,800                         | 24   |                    |
| T-222 | 2400(1)               | 29,400                                                    | 43,200                          | 36   |                    |
|       | R.T.(1)               | 107,600                                                   | 111,800                         | 25   |                    |
|       | 2400(1)               | 37,000                                                    | 52,500                          | 25   |                    |
|       | 2000(2)               | 89,200                                                    | 100,000                         | 10   |                    |
|       | 2400(2)               | 56,000                                                    | 61,300                          | 24   |                    |

1. Annealed one hour at 1650°C (3000°F) prior to testing  
2. Cold worked, stress relieved one hour at 2000°F.

the material was excellent in that tungsten inert gas welded butt joints and electron beam welded joints were ductile in bending at -200°F over a mandrel with a radius 1.8 times the sheet thickness.

The alloys of the invention were then tested to determine their creep properties at 2400°F in a vacuum of 10<sup>-8</sup> Torr. Alloy T-222 was similarly tested. The results are set forth in Table III below.

creep resistance as T-222 based on time to elongate 1 percent.

The high creep resistance exhibited by the alloys of this invention is attributable in part to the dispersed secondary phases of the carbides of the (Ta, W, Re, Mo, Hf, Zr)<sub>2</sub>C<sub>1-x</sub> type which inhibit dislocation motion, thereby decreasing creep rate. As noted hereinbefore the alloy of the present invention contains secon-

TABLE III

| Alloy | Test Temperature (°F) | Creep Properties<br>Annealed One Hour at 1650°C (3000°F) Prior to Testing |                  |                      |                | Time To Elongate (hrs.) |
|-------|-----------------------|---------------------------------------------------------------------------|------------------|----------------------|----------------|-------------------------|
|       |                       | Stress (psi)                                                              | Test Time (hrs.) | Total Elongation (%) |                |                         |
| A     | 2400                  | 15,000                                                                    | 192              | 0.26                 | over 200 (est) |                         |
| B     | 2400                  | 15,390                                                                    | 94               | 0.2                  | over 100 (est) |                         |
| C     | 2400                  | 15,000                                                                    | 90.9             | 1.03                 | 91             |                         |
| D     | 2400                  | 15,000                                                                    | 102              | 1.32                 | 90             |                         |
| E     | 2400                  | 15,000                                                                    | 554              | 2.53                 | 262            |                         |
| F     | 2400                  | 15,000                                                                    | 209              | 2.19                 | 115            |                         |
| T-222 | 2400                  | 15,000                                                                    | 235              | 4.7                  | 83             |                         |

All the alloys (A, B, C, D and E) exhibit improvement in resistance to creep deformation over alloy T-222 under the conditions of test listed in Table III. The improvement in resistance to creep is particularly marked in alloys A, B and E. Alloys A and B show substantially better properties than T-222 based on time to elongate 1 percent. Alloy E is more than three times as

secondary phases of dimetal carbides. Significant in this respect is the fact that the improved creep properties are associated only with the dimetal phases as illustrated in FIG. 2. Alloy E, which has outstanding creep properties was subjected to X-ray diffraction analysis of chemically extracted dispersed phases. The results are set forth hereinafter in Table IV.

35

TABLE IV

| NAS-56 (8W-1Re-0.7Hf-0.025C)<br>1 hr. at 1650°C/3000°F +<br>193 hrs. at 1315°C/2400°F<br>and 12,690 psi |           | NAS-56 (8W-1Re-0.7Hf-0.025C)<br>1 hr. at 1650°C/3000°F +<br>308 hrs. at 1315°C/2400°F<br>and 15,000 psi |           |
|---------------------------------------------------------------------------------------------------------|-----------|---------------------------------------------------------------------------------------------------------|-----------|
| d                                                                                                       | Intensity | d                                                                                                       | Intensity |
| 3.15                                                                                                    | VVV       | HfO <sub>2</sub>                                                                                        | 2.69      |
| 2.82                                                                                                    | VVVV      | HfO <sub>2</sub>                                                                                        | 2.62      |
| 2.69                                                                                                    | M         | HCP                                                                                                     | 2.47      |
| 2.62                                                                                                    | VVV       | (2.37Ta <sub>2</sub> C)                                                                                 | 2.37      |
| 2.47                                                                                                    | S         | HCP                                                                                                     | 1.82      |
| 2.37                                                                                                    | VS        | HCP                                                                                                     | 1.555     |
| 1.82                                                                                                    | MS        | HCP                                                                                                     | 1.405     |
| 1.555                                                                                                   | MS        | HCP                                                                                                     | 1.345     |
| 1.405                                                                                                   | MS        | HCP                                                                                                     | 1.315     |
| 1.345                                                                                                   | W         | HCP                                                                                                     | 1.300     |
| 1.315                                                                                                   | MS        | HCP                                                                                                     | 1.2355    |
| 1.300                                                                                                   | M         | HCP                                                                                                     | 1.183     |
| 1.2355                                                                                                  | W         | HCP                                                                                                     | 1.125     |
| 1.183                                                                                                   | W         | HCP                                                                                                     | 1.042     |
| 1.125                                                                                                   | W         | HCP                                                                                                     | 1.028     |
| 1.042                                                                                                   | M         | HCP                                                                                                     | 0.997     |
| 1.028                                                                                                   | W         | HCP                                                                                                     | 0.968     |
| 0.997                                                                                                   | MS        | HCP                                                                                                     | 0.941     |
| 0.968                                                                                                   | M         | HCP                                                                                                     | 0.929     |
| 0.941                                                                                                   | MW        | HCP                                                                                                     | 0.910     |
| 0.929                                                                                                   | MW        | HCP                                                                                                     | 0.897     |
| 0.910                                                                                                   | W         | HCP                                                                                                     | 0.867     |
| 0.897                                                                                                   | W         | HCP                                                                                                     | 0.844     |
| 0.867                                                                                                   | MS        | HCP                                                                                                     | 0.796     |
| 0.844                                                                                                   | M         | HCP                                                                                                     | 0.7875    |
| 0.796                                                                                                   | M         | HCP                                                                                                     | 0.796     |
| 0.7875                                                                                                  | VW        | HCP                                                                                                     | 0.776     |
| 0.796                                                                                                   | W         | HCP                                                                                                     |           |
| 0.776                                                                                                   | W         | HCP                                                                                                     |           |

Note: HCP with  $a_0 = 3.11$  Å  
 $c_0 = 4.95$  Å  
 $c/a = 1.59$   
 $(Ta, W, Re, Hf)_2 C_{1-x}$

HCP with  $a_0 = 3.11$  Å  
 $c_0 = 4.95$  Å  
 $c/a = 1.59$   
 $(Ta, W, Re, Hf)_2 C_{1-x}$

From the test results set forth hereinbefore it is clear that the stable secondary phase is that of the dimetal carbide. Since other test results show lattice constants  $a_0$  within the range of 3.10 Å. to 3.15 Å. and  $c_0$  within the range between 4.92 Å. and 4.96 Å. thus indicating very minor substitution of hafnium tungsten and rhenium for tantalum. This is in excellent agreement with the values of  $a_0 = 3.106$  Å. and  $c_0 = 4.945$  Å. reported for the compound  $Ta_2C$ .

As stated previously, the alloying components must be limited to 10 percent total substitutional solute components. The alloys (A, B, C, D and E) each contain less than 10 percent substitutional solute (W + Mo + Re + Zr + Hf) as opposed to approximately 12.5 W+Hf present in T-222. The amount of substitutional solute elements present in the alloy is an important consideration since fabricability is strongly affected by the amount of such solid solution strengtheners present. The more total strengthener present the less fabricable the alloy tends to be and therefore, more energy and heavier equipment is required to work the alloy. The substitution of rhenium for part of the tungsten in Alloys A, B and E effects an improvement in creep resistance. The addition of rhenium apparently increases the shear modulus of the matrix and decreases the diffusivity of matrix, thereby decreasing the creep rate.

The extraordinary effect of the rhenium addition in Alloy E is demonstrated by creep testing an alloy having the composition of Alloy F. Alloy F is similar in all respects to Alloy E except that in Alloy E 1 percent rhenium has been substituted for an equal weight of tungsten.

Comparing the results set forth in Table III for Alloys E and F it is seen that the time to elongate 1 percent is doubled by the substitution of 1 percent rhenium for 1 percent tungsten. This is quite surprising in view of the fact that the low temperature-short time properties such as yield strength and ductility (elongation) are substantially unaffected by this same substitution. Thus the preferred alloy contains about 1 percent rhenium.

The element oxygen is undesirable in the alloys of this invention since the oxides are formed in a particle size which is too large to effectively pin dislocations. Further, the oxygen removed hafnium from solution and reduces the amount available for reaction with the carbon and nitrogen. Accordingly, oxygen in these alloys is preferably restricted to an amount of 100 parts per million or less.

Thus, there have been described tantalum-base alloys having exceedingly useful properties and which are suitable for application at elevated temperatures in a vacuum environment.

It will be understood by those skilled in the art that although the invention has been described in connection with preferred alloys, modifications and variations may be employed without departing from the underlying spirit and scope of the invention.

I claim as my invention:

1. A tantalum base alloy particularly adapted for use at elevated temperatures under high vacuum consisting essentially of, by weight, from about 4 percent to about 8.5 percent tungsten, from about 0.5 percent to about 3.0 percent of at least one metal selected from the group consisting of molybdenum, rhenium and mixtures thereof, the molybdenum when present being within the range of up to about 1.25 percent and the

rhenium, when present being within the range of up to about 3 percent, up to about 1.5 percent of at least one metal selected from the group consisting of hafnium, zirconium and mixtures thereof, the hafnium, when present being within the range of up to about 1.5 percent and the zirconium when present being within the range of up to about 0.75 percent, from about 0.01 percent to about 0.04 percent of at least one element selected from the group consisting of carbon, nitrogen and mixtures thereof, the carbon, when present being within the range of traces to about 0.03 percent and the nitrogen when present being within the range traces up to about 0.03 percent and the balance tantalum with incidental impurities, the alloy being fabricable while having a DBTT below room temperature and the alloying elements being selected within the ranges stated to produce a microstructure characterized by exhibiting a dispersed secondary phase of a dimetal carbide of the  $(Ta, W, Mo, Re, Hf, Zr)_2 C_{1-x}$  type, is substantially free of monometal carbides and which alloy exhibits excellent creep properties.

2. An alloy as set forth in claim 1 wherein tungsten is present in amounts of from 4 to 8 percent, molybdenum is present in amounts of from 0.5 to 1.25 percent, rhenium is present in amounts of from 0.5 to 1.25 percent, hafnium is present in amounts of from 0.1 to 1.5 percent and nitrogen is present in amounts of from 0.01 to 0.03 percent as a partial substitute for carbon.

3. An alloy as set forth in claim 1 wherein tungsten is present in amounts of from 5.5 to 5.8 percent, molybdenum is present in amounts of from 0.6 to 0.9 percent, rhenium is present in amounts of from 1.4 to 1.6 percent, hafnium is present in amounts of from 0.2 to 0.3 percent, zirconium is present in amounts of from 0.1 to 0.2 percent, carbon is present in an amount of from 0.02 percent and nitrogen is present in an amount of about 0.02 percent.

4. An alloy as set forth in claim 1 wherein about 6.3 to 7.2 percent of tungsten is present, molybdenum, when present amounts to about 0.7 to 1 percent, rhenium, when present, amounts to about 1.4 to 1.6 percent, about 0.2 to 0.3 percent zirconium is present, about 0.4 to 0.6 percent hafnium is present, about 0.02 percent nitrogen is present, and traces to about 0.02 percent carbon is present.

5. An alloy as set forth in claim 1 wherein from 6.8 to 7.2 percent tungsten is present, from 1.4 to 1.6 percent rhenium is present, about 0.2 to 0.3 percent zirconium is present and about 0.02 percent nitrogen is present as a partial substitute for carbon.

6. An alloy as set forth in claim 1 wherein from 6.8 to 7.2 percent tungsten is present, from 0.7 to 1 percent molybdenum is present, from 0.2 to 0.3 percent zirconium is present and about 0.02 percent nitrogen is present as a partial substitute for carbon.

7. An alloy as set forth in claim 1 wherein from 6.3 to 7.2 percent tungsten is present, from 0.7 to 1 percent molybdenum is present, from 0.2 to 0.3 percent zirconium is present, from 0.4 to 0.6 percent hafnium is present, about 0.02 percent carbon is present and about 0.02 percent nitrogen is present.

8. A highly workable tantalum-base alloy having exceptional resistance to creep deformation consisting essentially of, by weight, from about 7 to 8.5 percent tungsten, from 0.5 to 1.5 percent rhenium, from 0.5 to 1.25 percent hafnium, from 0.02 to 0.03 percent carbon and the balance essentially tantalum with small amounts of impurities, said alloying components being selected within the ranges stated to produce a micro-

11

structure exhibiting a dispersed secondary phase of a dimetal carbide of the  $(\text{Ta}, \text{W}, \text{Mo}, \text{Re}, \text{Hf}, \text{Zr})_2 \text{C}_{1-x}$  type and which is substantially free of mono-metal carbides.

9. The alloy of claim 8 wherein tungsten is present in

12

an amount of about 8 percent, rhenium is present in an amount of about 1 percent, hafnium is present in an amount of about 0.7 percent and carbon is present in an amount of about 0.025 percent carbon.

\* \* \* \* \*

5

10

15

20

25

30

35

40

45

50

55

60

65